

## UNITED STATES PATENT OFFICE

2,149,531

## PROCESS FOR TREATING MINERAL OILS

Wilbert B. McCluer and Merrell R. Fenske, State College, Pa., assignors to Pennsylvania Petroleum Research Corporation, a corporation of Pennsylvania

No Drawing. Application December 26, 1933,  
Serial No. 704,052

4 Claims. (CL. 196—13)

This invention pertains generally to the separation of materials into components and pertains particularly to the separation of mineral oils into parts or fractions having different characteristics.

In accordance with this invention crude petroleum or products thereof and particularly lubricating oils are separated into various components by first dissolving the material to be treated in a suitable solvent and then fractionally precipitating the dissolved oil from said solvent.

In a simple extraction process of the prior art, equilibrium between the dissolved and undissolved oil may be approached from either the low temperature or high temperature side. If equilibrium is approached from the low temperature (or constant temperature) side, the process is merely one of extraction in its usual form. If equilibrium is approached from the high temperature side, an excess of oil will be dissolved and as the temperature is lowered to the point at which final separation is effected, the excess oil dissolved in the solvent layer will be precipitated. The results in either case will be identical provided sufficient time is allowed for equilibrium to be established between dissolved and undissolved oil.

Results comparable to the second case above may be obtained by dissolving all or a large portion of the oil in one solvent (called solvent A) and then precipitating a part of said dissolved oil by the addition to the solution of a suitable second solvent (called solvent B), or results comparable to the first case above may be obtained by treating the oil with a mixture of solvents A and B in the first instance.

In other words, precipitation may be effected either by reducing the temperature or by the addition of a suitable second solvent, and in either case as long as the process is single stage and equilibrium has been established between the solvent layer and the oil layer, the results will be substantially identical to those obtained by simple extraction without precipitation.

Fractional precipitation, on the other hand, is distinctly different from the foregoing. Fractional precipitation is effected by first dissolving a desired percentage (up to 100 per cent) of the oil in a suitable solvent and then precipitating (either by temperature reduction or the addition of a second solvent, or both) and removing successive amounts of the dissolved oil. In other words, each precipitated oil layer is removed prior to further precipitation.

Fractional precipitation is particularly adapted to the production of several different qualities

of oil. This feature follows directly from the fact that a large number of fractions can be obtained from a given oil. Since both the viscosity and quality of the different fractions vary, it is possible to produce oils of practically any grade and quality by blending the various fractions in the desired proportions.

Fractional precipitation is more efficient than simple single stage extraction. The increased efficiency may be explained as follows: In single stage extraction or precipitation, a relatively large percent of highly paraffinic materials must be present in the solvent layer at all times in order to maintain equilibrium between the dissolved and undissolved oil and the amount of these highly paraffinic dissolved oils is greatest when the quality of the raffinate is highest. If, on the other hand, successive precipitates are removed from the system, the dissolved oil is in equilibrium with the successively lower quality undissolved oil and hence the amount of highly paraffinic material dissolved at the end of the fractional precipitation process is reduced considerably. In other words, it is possible to obtain a higher yield of improved oil of a given quality by fractional precipitation than by single stage extraction or precipitation, or similarly for a given yield the quality of the improved oil is higher when it is produced by fractional precipitation than when it is produced by single stage extraction or precipitation.

As specific examples of these methods, assume a given oil is dissolved completely in solvent A at temperature T. If the temperature is now reduced to T', a definite quantity of oil (Q') will be precipitated. If this precipitated oil is not removed from the system and the temperature is further reduced to T" a second definite quantity of oil will be precipitated and the total quantity of undissolved (or precipitated) oil will be Q". Comparing this with extraction, let it be assumed that the same oil is treated with the same ratio of solvent A at the temperature T'. Since the conditions of temperature, solvent, and solvent-oil ratio are identical, when equilibrium is established the amount of undissolved oil will be Q' and this oil will have properties comparable to that of the oil Q' in the preceding case.

Similarly, the results obtained by precipitation at temperature T" will be comparable to those obtained by extraction at this temperature provided similar conditions obtain. Hence, the results obtained by single stage extraction or by single stage precipitation will be substantially identical under similar processing conditions.

In the previous conditions of precipitation when the temperature was  $T'$  and the quantity of oil precipitated was  $Q'$  the quality and quantity of the oil were independent of the process employed. If, however, the quantity of oil  $Q'$  is removed when the precipitation temperature is  $T'$  and the temperature is then reduced to  $T''$ , a product  $Q_r$  will be obtained which will be quite different from the product  $Q''$ . The product  $Q_r$  will not only be different from  $Q''$  but on the basis of the laws of equilibrium distribution should the products  $Q_r$  and  $Q''$  be combined, the properties of such combined products will be different from the properties of  $Q''$ . These conditions will prevail as long as successive amounts of oil are precipitated.

Fractional precipitation may be effected by reduction in temperature as indicated above or by the addition of successive amounts of a second solvent (solvent B) to a solution of oil dissolved in a first solvent (solvent A) or dissolved in a solvent mixture consisting of solvent B and solvent A. A similar relation exists between single stage extraction, single stage precipitation, and fractional precipitation when oil is precipitated by the addition of a second solvent as that which has been indicated previously for the case when oil is precipitated from an oil-solvent solution by reduction in temperature.

30 In these processes solvent B is so chosen that the solubility of oil in mixtures of solvents A and B is less than the solubility of oil in solvent A at the same temperature.

This invention pertains more particularly to fractional precipitation by the addition of a second solvent, wherein the solvents are combined efficiently for this particular purpose. For instance, we find that same particular solvent X may have a greater selectivity than some other solvent Y when fairly low percentage amounts of oil are to be dissolved. However, the selective characteristics of the same two solvents may be reversed when larger percentage amounts of the same oil are to be dissolved so that when fairly high percentage amounts of oil are dissolved solvent Y is more selective than solvent X.

For instance, sulphur dioxide has a higher selectivity than nitrobenzene when low percentage amounts of oil are to be dissolved. On the other hand, when high percentage amounts of oil are to be dissolved, nitrobenzene has a higher selectivity than sulphur dioxide.

Similarly the selectivity of pyridine increases with increase in the amount of oil dissolved whereas the selectivity of methyl cellosolve decreases with increase in the amount of oil dissolved. Both of these solvents are excellent solvents for solvent extraction, subject, however, to the limitations set forth.

60 This invention is directed to the utilization of the foregoing solvents in solvent extraction in a manner to overcome the foregoing limitations making it possible to employ each solvent over a range in percentage of oil dissolved in which said solvent is more selective.

65 This is accomplished by progressively varying the relative concentrations of two solvents of the foregoing characteristics in accordance with the quantity of oil in solution.

70 This can be carried out very effectively by resorting to fractional precipitation methods employing the solvent whose selectivity increases with the amount of oil in solution to originally dissolve the oil and then employing the solvent whose selectivity increases with decrease in

amount of oil dissolved to precipitate oil from solution in said first solvent.

The fact that the selective rating of a solvent depends not only on the characteristics of the solvent but also on the amount of oil dissolved is now fairly well established. We have discovered that it is more efficient (from the standpoint of economy in degraded oil) to employ different solvents in the extraction of an oil, each solvent being employed over the range in 10 percentage of oil dissolved in which it is most selective. We also find that such a condition can be approached by means of a process of fractional precipitation in which oil is precipitated by the addition of a second solvent. 15

As an example of the latter, all or a large part of the oil may be dissolved in solvent Y and successively precipitated by the addition of regulated amounts of solvent X. Since at the beginning of the step by step precipitation the solvent 20 mixture is composed chiefly of solvent Y and a large part of the oil is in solution, the selectivity of the mixed solvents is high, since solvent Y predominates. As the step by step precipitation proceeds by the addition of regulated amounts 25 of solvent X, lesser quantities of oil remain dissolved in the solvent mixture and the influence of solvent X becomes greater and greater such that when a fairly large amount of oil has been precipitated the concentration of solvent X relative to solvent Y is high and the solvent mixture continues to be highly selective since only small amounts of oil remain dissolved. Thus by a series of combinations of solvents X and Y at the beginning of which series the concentration 30 of solvent Y is relatively high and the concentration of solvent X is relatively low and in which series the concentration of solvent Y decreases and the concentration of solvent X increases as the step by step precipitation 35 proceeds, it is possible to have an optimum selectivity throughout the process of fractional precipitation.

Although the process of fractional precipitation is applicable to the processing of oils 45 of all types including those from the midcontinent and western fields in which the problem is principally one of deasphaltization to remove products of extremely low lubricating value, it is particularly applicable to the processing of petroleum oils of Pennsylvania grade which contain 50 no or at most only minute quantities of deleterious substances and substantially all the components of which are suitable for lubrication purposes. Thus the problem in improving a Pennsylvania oil for automotive purposes is not 55 one of removing substances which would be deleterious to an automobile motor, such as asphalt, but becomes one of improving the flash and fire points, the reduction in viscosity difference between 100° F. and 210° F. and the reduction of Conradson carbon residue. For instance, it is found that when working with lubricating stock of Pennsylvania grade since such lubricating stock is already of high quality it is possible 60 to produce from the original oil 10 to 15% of very high grade improved oil and yet not seriously affect the physical characteristics of the remaining 65 to 90% by employing at the beginning of the process a solvent having a high 65 selectivity when high percentage amounts of oil are dissolved.

As an example of the above process, one volume of bright stock was mixed with six volumes of pyridine. To this mixture a small amount of 75

methylcellosolve was added and the mixture was stirred for ten minutes at 90° F. With constant stirring the temperature was brought down to 79° F. and the stirring continued at this temperature for twenty minutes. The mixture was then allowed to settle for two hours at this temperature and then the layers were separated.

After separation of the two layers, the precipitated or residual layer (raffinate) was treated in the usual way to remove the solvent from it and this solvent-free oil was tested for its various physical properties.

A small amount of the solvent layer containing dissolved oil was set aside for tests while the remainder was used as stock for the next precipitation.

The next precipitate was formed by adding to the stock a second small amount of methylcellosolve. After stirring the mixture was allowed to settle at the same temperature into a two layer system as before and the precipitate was removed.

This procedure was repeated seven times. In each step of the fractional precipitation process approximately eight to thirteen per cent of the original oil was precipitated and the total amount precipitated was 71.6 per cent.

Results of a similar character are shown in condensed form in the following table:

30

30

methylcellosolve was added with thorough agitation and approximately 7.9 per cent of the oil was precipitated. This precipitated oil had a 210° F. viscosity at 249 Saybolt seconds, and A. P. I. gravity of 28.4°, and a viscosity index of 111. From these data, it is evident that a considerably improved product has been obtained.

A second quantity of methylcellosolve (approximately 0.15 volume) was then added with thorough agitation to the remaining oil dissolved in the solvent and a second quantity of precipitated oil (9.2 per cent of the original oil) was obtained. This fraction had a 210° F. viscosity of 194 Saybolt seconds and an A. P. I. gravity of 28.5° and a viscosity index of 109.

A total of eight different products (see Table I) were obtained from the bright stock by this procedure, seven of them being precipitated oils of improved characteristics and one of them being degraded oil. All of the precipitated oil fractions had physical properties superior to the original oil and a total yield of 71.6 per cent of improved oil was separated.

The above data were obtained for the primary purpose of indicating the improvements which can be made in oils of Pennsylvania grade and do not indicate the maximum efficiency which can be obtained through the utilization of properly designed and operated equipment. The yield

TABLE  
*Fractional precipitation of bright stock*

| Run No. | Percent of methylcellosolve in solvent | Oil                    | Percent extracted based on— |                       | Viscosity |         | Grav-<br>ity<br>°A.P.I. | Speci-<br>fic<br>gravity<br>at<br>20° C. | Refrac-<br>tive<br>index<br>at<br>20° C. | Vis-<br>cosity<br>index | Gravity<br>index | A. S. T. M. | Color | Pour<br>point,<br>°F. |
|---------|----------------------------------------|------------------------|-----------------------------|-----------------------|-----------|---------|-------------------------|------------------------------------------|------------------------------------------|-------------------------|------------------|-------------|-------|-----------------------|
|         |                                        |                        | Original<br>charge          | Total<br>in<br>system | 210° F.   | 100° F. |                         |                                          |                                          |                         |                  |             |       |                       |
| 40      |                                        | Original bright stock. | 100                         | 100                   | 153.9     | 2452    | 26.4                    | 0.8938                                   | 1.496                                    | 99.5                    | 106              | 8           |       | 25                    |
| A-1     | 4.0                                    | Precipitate            | 7.9                         | 7.9                   | 249.3     | 4058    | 28.4                    | 0.8831                                   | 1.488                                    | 111                     | (Extr.)          | 8           | Dark  | 30                    |
|         |                                        | Extract                | 92.1                        | 92.1                  | 147.7     | 2382    | 26.1                    | 0.8955                                   | 1.497                                    | 97                      |                  |             |       |                       |
| 45      | 6.1                                    | Precipitate            | 9.2                         | 10.0                  | 194.4     | 2950    | 28.5                    | 0.8825                                   | 1.437                                    | 109                     | 119              | 8           | Dark  | 25                    |
|         |                                        | Extract                | 82.9                        | 90.0                  |           |         |                         |                                          |                                          |                         |                  |             |       |                       |
| A-3     | 9.0                                    | Precipitate            | 13.1                        | 16.8                  | 162.2     | 2305    | 28.6                    | 0.8818                                   | 1.487                                    | 108                     | 116              | 8           | Dark  | 25                    |
|         |                                        | Extract                | 69.8                        | 84.2                  | 139.0     | 2313    | 25.3                    | 0.9003                                   | 1.500                                    | 92                      |                  |             |       |                       |
| A-4     | 12.5                                   | Precipitate            | 11.5                        | 16.5                  | 141.2     | 1915    | 28.6                    | 0.8815                                   | 1.487                                    | 106                     | 115              | 8           | Dark  | 25                    |
|         |                                        | Extract                | 58.3                        | 83.5                  |           |         |                         |                                          |                                          |                         |                  |             |       |                       |
| 50      | 16.5                                   | Precipitate            | 9.8                         | 16.8                  | 129.6     | 1692    | 28.5                    | 0.8821                                   | 1.487                                    | 105                     | 113              | 8           | Dark  | 30                    |
|         |                                        | Extract                | 48.5                        | 83.2                  | 144.4     | 2727    | 23.7                    | 0.9004                                   | 1.505                                    | 84                      |                  |             |       |                       |
| A-6     | 22.9                                   | Precipitate            | 10.5                        | 21.7                  | 120.3     | 1551    | 28.2                    | 0.8838                                   | 1.488                                    | 104                     | 111              | 8           | Dark  | 20                    |
|         |                                        | Extract                | 38.0                        | 78.3                  |           |         |                         |                                          |                                          |                         |                  |             |       |                       |
| A-7     | 33.0                                   | Precipitate            | 9.6                         | 25.2                  | 114.9     | 1504    | 27.8                    | 0.8861                                   | 1.490                                    | 100                     | 109              | 8           | Dark  | 25                    |
|         |                                        | Extract                | 28.4                        | 74.8                  | 177.7     | 4845    | 20.5                    | 0.9288                                   | 1.514                                    | 66                      |                  |             |       |                       |

Precipitation temperature: 79° F.

Solvent: Pyridine.

Precipitant: Methylcellosolve.

Solvent to oil volume ratio at start: 6.

The results of our investigation show that by processing a lubricating stock of Pennsylvania grade with selective solvents of the above character and in the above manner, the flash and fire points, the A. P. I. gravity, and the viscosity index of the precipitates increase from the last toward the first precipitates and the Conradson carbon residue decreases from the last to the first precipitates.

In the example under consideration, the final extract comprised 28.4 per cent of the original oil with a viscosity index of 66, which compares very favorably with lubricating oils from the midcontinent or western fields.

The bright stock of the above table was completely dissolved in six volumes of pyridine at 79° F. Twenty-five hundredths of a volume of

of products having a definite degree of improvement may be increased to a large extent dependent upon the efficiency of the processing equipment.

Although the highest improvement in viscosity index of the precipitates of Table I is 11.5 points, it is to be pointed out that the first precipitate had a viscosity at 210° F. of 249.3 Saybolt Universal and that a high degree of improvement was actually effected.

Oils of equal viscosity index but of different 210° F. viscosity have considerably different relative viscosity-temperature coefficients than would be anticipated from the numerical value of the viscosity index. As a specific example, consider the case of an oil having a 210° F. viscosity of 220 seconds Saybolt and a viscosity index of 125. Offhand, it might be assumed that the degree of improvement in this oil is similar to that in an oil having a 210° F. viscosity of, say, 63 seconds Saybolt and a viscosity index of

125. However, such is not the case since the theoretical maximum viscosity index of an oil having a 210° F. viscosity of 220 seconds Saybolt is only 150 while that of a 63 second oil is 200. 5 It is evident that in one case the oil has been improved to within 50 per cent of its theoretical maximum while in the case of the lighter oil the degree of improvement is only 25 per cent of the theoretical maximum.

10 The theoretical maximum referred to above indicates that degree of improvement in an oil at which the viscosities at 100° F. and 210° F. are equal.

15 From the foregoing it will be seen that a very considerable improvement has been effected not only in the first precipitate but in many of the succeeding precipitates.

20 From the foregoing it will be seen that a mineral oil and particularly one of Pennsylvania grade may be divided into any desired number 25 of portions having different viscosity-temperature coefficients and different viscosities at the same temperature and since both the viscosity and quality of the different fractions vary, it is possible to produce oils of practically any grade and quality by blending the various fractions in any desired proportions.

30 It is more difficult to improve a petroleum oil of Pennsylvania grade due to its original high quality and such oils may be very substantially improved by the process herein. The process, however, might be employed to effect improvement in other oils such as those of naphthenic or asphaltic characteristics.

35 While we have particularly described means for effecting precipitation, it is to be understood that such means might be combined or other means might be employed alone or in conjunction with one or more of the means specifically referred to herein. For instance, it is possible 40 to cause step by step precipitation by reducing the solvent concentration, for instance, by vaporization of solvent through any means known in the art such as the reduction of the total pressure on the solution with or without the application of heat.

45 In the claims the term "lubricating oil" when referred to is intended to mean an oil of a viscous character, that is, of the order of 35 Saybolt seconds at 210° F. or above.

50 The particular description herein is by way of illustration and it is therefore to be understood that changes, omissions, additions, substitutions, and/or modifications may be made without departing from the spirit of the invention which is intended to be limited only as required by the prior art.

55 For instance, it is not necessary to remove all of the precipitate formed in each step and a part only thereof might be separated in one or

more of the steps without departing from the invention.

60 By a precipitating solvent is meant a solvent which when added to a solvent-oil solution forms with the solvent of the solution a solvent mixture of lesser solubility for the oil.

65 The successive precipitations need not be accomplished by the addition of the same solvent throughout, but a second or a series of solvents may also be employed for this purpose.

70 The term solvent in its broader significance includes any compound or mixture of compounds having desired characteristics whether in the vapor, liquid, and/or solid phase.

75 We claim:

1. A process comprising dissolving a lubricating oil in pyridine, precipitating oil from said solution in steps by successively introducing into said solution desired quantities of methylcellosolve, and removing precipitate formed after each addition of methylcellosolve and prior to the next addition of methylcellosolve.

2. A process comprising dissolving a lubricating oil in pyridine, precipitating oil from said solution in steps by successively introducing into said solution desired quantities of methylcellosolve, removing precipitate formed after each addition of methylcellosolve and prior to the next addition of methylcellosolve, and blending selected precipitated fractions.

3. In a process for extracting a lubricating oil with a mixture of solvents for components of the oil, the steps of employing a plurality of selective solvents in said solvent mixture one of which increases in selectivity as the amount of oil in solution increases and another of which increases in selectivity as the amount of oil in solution decreases, forming two liquid phases of oil and solvent mixture in each of a series of stages in which the amount of oil in solution in said solvent mixture varies progressively from one stage to the next, and increasing the proportion of said second solvent to said first solvent in said solvent mixture as the amount of oil in solution in said solvent mixture decreases and vice versa.

4. In a process for extracting a lubricating oil with a mixture of solvents for components of the oil, the steps of employing a plurality of selective solvents in said solvent mixture one of which increases in selectivity as the amount of oil in solution increases and another of which increases in selectivity as the amount of oil in solution decreases, forming extract and raffinate phases from said oil and solvent mixture, and increasing the proportion of second solvent to first solvent with increase in the proportion of raffinate to extract and vice versa.

WILBERT B. MCCLUER.

MERRELL R. FENSKE.

60